

May 19, 1936.

A. R. STARGARDTER

2,041,029

## METHOD OF TREATING METAL

Filed Sept. 4, 1931

3 Sheets-Sheet 1



May 19, 1936.

A. R. STARGARDTER

2,041,029

## METHOD OF TREATING METAL

Filed Sept. 4, 1931

3 Sheets-Sheet 2



## INVENTOR

*A.R. Stargardter*

BY

T. F. Bowen

**ATTORNEY**

May 19, 1936.

A. R. STARGARDTER

2,041,029

METHOD OF TREATING METAL

Filed Sept. 4, 1931

3 Sheets-Sheet 3

Fig. 9



INVENTOR  
A. R. Stargardter  
BY  
T. P. Bourne,  
ATTORNEY

## UNITED STATES PATENT OFFICE

2,041,029

## METHOD OF TREATING METAL

Albert R. Stargardter, Newark, N. J., assignor to  
 Gillette Safety Razor Company, Boston, Mass.,  
 a corporation of Delaware

Application September 4, 1931, Serial No. 561,183

6 Claims. (Cl. 148—10)

An object of my invention is to treat continuous lengths of magnetizable metal, such as hardened or annealed steel strips, (or ferrous-alloys), in such a way as to produce substantial uniformity of a desired character throughout the length of the strip, such as hardness and/or temper, or an annealed condition, in a simple and relatively inexpensive manner.

Another object of my invention is to control the treatment of a metal strip as it travels in accordance with desired characteristics, such as hardness and/or temper or an annealed condition, of a piece of the same or a similar strip that has been hardened and/or tempered, or annealed, and which is used as a "standard", whereby the strip being treated will have substantially throughout characteristics similar to those of the standard piece and will be substantially free from variations from the latter.

Another object of my invention is to cause control of the heat applied to a traveling steel strip by utilizing definite characteristics in portions of the strip, or variations or changes therefrom in the metallurgical characteristics within other portions of the strip itself, whereby to retain a substantially definite or predetermined heat applied to the strip in the heating zone, if required, or to automatically increase or decrease the heat applied to the strip in such zone as may be required, as the strip travels, to cause the resulting product to be substantially uniform throughout its length according to a predetermined standard.

Any change in the microstructure of steel or any other ferrous-alloy is accompanied by a change in the electrical permeability of the metal. For example, a steel which has been quenched from 1600° F. will possess less permeability than if it had been quenched from 1500° F. The same steel quenched from 1500° F. will possess less permeability than if it had been quenched from 1400° F., at the same cooling rate.

These phenomena are due to the fact that in a given steel or steels identical in composition, microstructure, and pre-natal history, the higher the quenching temperature the greater the amount of carbides held in solid solution. The electrical permeability is inversely proportional to the amount of carbides in solid solution. This principle is also true for annealed steels.

A steel annealed from 1500° F. at a certain cooling rate will possess greater permeability than the same steel or steels identical in composition and pre-natal history annealed from 1400° F., since the steel annealed from 1500° F. will have less carbide in solid solution than that annealed from 1400° F.

It also follows from the above that in the case of either hardened or annealed steels (or ferrous-alloys) that the electrical permeability is inverse-

ly proportional to the cooling rate. Identical steels cooled at the rate of one degree per second will have greater permeability than those cooled at the rate of 40° per second, etc. Thus water-quenched steels have less permeability than similar steels oil quenched. 5

It is also true that in the case of steels identical in composition and pre-natal history the electrical permeability varies inversely with the net carbon content. 10

In accordance with my invention, I utilize the electrical permeability of a "standard" piece of magnetizable metal which has been predetermined as to the desired characteristics to cause the strip to be heat-treated, namely, to be hardened and/or tempered, or annealed, in substantial correspondence as to desired characteristics in the treated strip of those in the standard strip. 15

In carrying out my invention, I provide an electrically heated apparatus through which the strip to be heat-treated is propelled and electrical devices through which the heat-treated strip travels. Said devices are adapted to react to electrical permeability changes or variations in such strip as compared to a standard piece of similar material in said devices to register, indicate and/or control automatically any such changes or variations from the standard piece to cause the heating apparatus to apply a required temperature to a traveling strip, such as maintaining a given heat or reducing such heat, for a required period, and for restoring a higher heat as may be required, to cause the strip to be heat-treated so that its desired characteristics will, throughout its length, substantially correspond to those of the standard piece. 30

In a particular embodiment of my invention as illustrated in the accompanying drawings, I provide an electrically heated induction furnace having an automatic control switch in its supply line, means to continuously propel a metal strip through the furnace, means to quench the heated strip, a pair of transformers respectively having passageways for the strip under treatment and for a piece of "standard" metal, the secondaries of the transformers having opposite windings electrically opposed, in an electrically balanced circuit including a galvanometer, a mirror operated by the galvanometer, a photo-electric cell to receive a light beam from the mirror, a lens system serving to focus the light emanating from the mirror upon the photo-electric cell window, and a circuit controlled by the photo-electric cell including devices to operate the aforesaid switch. The arrangement described is such that a "standard" metal piece will be placed in one transformer and the strip after emerging from the quenching and/or tempering means will travel through the other transformer. If the last named portion of the strip corresponds to the standard piece 55

- the light beam from the galvanometer mirror will rest upon the photo-electric cell, causing the circuit through the furnace to remain closed for standard operation. Should the furnace temperature rise and change the then existing characteristics of the quenched strip a differential will occur in the circuit of the transformer secondaries causing the galvanometer to operate the mirror to remove the light beam from the photo-electric cell, thereby causing the latter to cease functioning and the circuit through the furnace will be broken. When the furnace drops to an appropriate temperature (and the characteristics of the quenched strip and the "standard" piece correspond) the galvanometer circuit will balance and the galvanometer will operate and cause the light beam to again fall on the cell to cause closing of the furnace switch to restore heating of the latter. In this way the temperature of the furnace may be maintained at such a condition as will produce a substantially uniform hardening of the strip throughout its length in substantial correspondence with the "standard" piece.
- 25 My invention also comprises novel details of improvement that will be more fully hereinafter set forth and then pointed out in the claims.
- Reference is to be had to the accompanying drawings, wherein
- 30 Fig. 1 is a side elevation of an apparatus adapted to carry out my invention;
- Fig. 2 is a plan view of the apparatus;
- Fig. 3 is a sectional view partially on line 3, 3 in Fig. 2;
- 35 Fig. 4 is a cross section on line 4, 4 in Fig. 3;
- Fig. 5 is a detail view illustrating the galvanometer and photo-electric cell in operative relation;
- Figs. 6, 7, and 8 are detail views illustrating 40 various positions of the galvanometer mirror with respect to the photo-electric cell, and
- Fig. 9 is a diagrammatic view of the electrical devices for controlling the furnace temperature.
- Similar numerals and letters of reference indicate corresponding parts in the several views.
- Upon a suitable frame 1 is mounted an electric induction furnace 2 through which a strip A of metal, such as relatively thin steel, is to be propelled in a continuous way. The furnace illustrated comprises a muffle 3 of suitable metal, shown in tubular form, open at both ends for the passage of strip A. The muffle is enclosed in insulation 4 around which is a conductor coil 5 that is enclosed in insulation 6. Said parts are shown enclosed in an outer protective casing 7, (Figs. 3 and 4). The coil 5 is shown connected with conductors 8 and 9 leading from a high frequency converter 10 of any desired construction, to be supplied from an A. C. line source 11.
12. The muffle will be heated by induction from the coil 5 for heating the strip A as it travels. The coil 5 is shown in tubular form and connected with rubber hose at 5a, 5b, to be supplied with running water, cold water running through the tubular coil thus keeping the coil cool. Said strip may be supplied on a reel 13 and wound on a take-up reel 14 in a well known way. Any suitable propelling means for strip A may be provided. I have illustrated a pair of opposed rolls 15 and 16 suitably journaled for gripping and feeding the strip. The roll 15 is shown provided with a gear 17 in mesh with a worm 18 operative by chain 19 on sprockets 20, 21 driven by a motor 22 to propel the strip A through the furnace at a substantially constant speed of travel.

At 23 and 24 are cooling plates between which the heated strip A passes in a quenching zone from the furnace or heater for chilling or quenching the heated strip. A cooling water tank is indicated at 25 on plate 24. The heated strip will be quenched in a well known way by passing between the chilling plates.

At 26 and 27 are a pair of step-down transformers having primary windings 28 and 29 in series in a circuit, shown including conductors a, b, and c, (Figs. 1 and 9). A switch at d permits connection of said conductors with the A. C. supply line conductors at e. An adjustable resistance is indicated at f for the conductor c. (Fig. 9). The secondary windings 28' and 29' of said transformers are oppositely wound and are thus electrically opposed, their terminals being shown connected by a conductor 30, the other terminals of the secondaries 28' and 29' being respectively connected by conductors 31 and 32 with the movable coil 33 of alternating current galvanometer 34. The said secondaries have no permanent cores and the transformers are so constructed as to be in perfect electrical balance until strip A has passed through an electrical field in secondary 28' and a standard metal piece B is placed to rest in an electrical field in secondary 29', serving as cores within the secondaries. The primaries and secondaries have passageways 28'' and 29'', respectively, to receive the strip A and standard piece B. The circuit through coil 33 of the galvanometer field circuit is controlled by switch 37 connected with the A. C. supply line 38 to receive suitable electric current, (Fig. 9). A mirror or reflector 41 is connected with movable coil 33 so as to be rotated thereby. At 42 is a light source, such as an electric lamp, shown located within the casing 40, to cast a light beam on the mirror 41. The lamp 42 is shown enclosed within a shield 43 having an aperture 44 for the light beam. Different angular positions of the mirror, on one side or the other of a predetermined position, such as in Fig. 7, are utilized to indicate and/or control the flow of current through the coil 5 of the furnace in accordance with difference in characteristics between the standard piece B in transformer 27 and the portion of strip A passing through the transformer 26. The arrangement is such that when the mirror is in the position shown in Fig. 7, the circuit for coil 5 should be closed and if the temperature of the furnace should unduly rise, the strip A will be so heated as to cause a difference in characteristics between the portion of the strip passing through the transformer 26 and the standard piece B to cause unbalancing of the circuit through the secondaries of the transformers, whereupon the coil 33 will rotate the mirror to an angular position at one side of the position of Fig. 7, such as to the position shown in Fig. 6, and the circuit for the coil 5 will be broken automatically. When the temperature of the furnace has dropped so that the characteristics of the portion of the strip passing through the transformer 26 compares with the characteristics of the standard piece B, the galvanometer coil 33 will operate to return the mirror to its normal position, such as in Fig. 7, whereupon the circuit through the coil 5 will be closed automatically.

If a still greater divergence in the metallurgical characteristics of the pre-treated strip should exist so that the portion passing through transformer 26 shows greater permeability than was the case in that portion giving rise to the mirror position in Fig. 7, the mirror 41 will move still

farther to the left (to position shown in Fig. 8), and the furnace heating circuit will remain closed until the traveling strip, due to this heating, will regain properties of the strip causing the mirror 5 position shown in Fig. 6. My invention includes means to automatically control the circuit through the heater coil 5, in accordance with the position of the mirror 41. Devices for such purposes are arranged as follows:—

10 At 45 is a photo-electric cell supported by frame 1 in position to receive the light beam reflected from the mirror.

The circuit 46 of the photo-electric cell through the amplifying tube 47 is utilized to control the flow of current through the coil 5 of the furnace by the operation of a relay or magnetic contactor 48 to control the A. C. supply line 12, (Fig. 9). To obtain the desired power to operate the magnetic contactor 48, I have illustrated a 20 transformer 49 whose secondary winding 50 is included in the circuit 51 of the photo-electric cell and whose primary winding 52 is supplied with suitable A. C. current through the switch controlled line 53. A grid-leak *g*, a fixed condenser 25 *h* and a potentiometer *i* are shown for the photo-electric cell circuits. A relay 54, as controlled by a solenoid coil 55 in the circuit 51 of the photo-electric cell, may be normally kept open by a spring 56. When the light beam is upon the 30 photo-electric cell, sufficient power from photo-electric cell, amplified through the system shown, will energize coil 55 to cause the relay 54 to close the line 57 through the coil 58 of the normally open relay contactor 48 to cause the latter to close the circuit of line 11, 12 to the converter to supply current to coil 5 of the furnace. The coil 58 35 may be a solenoid coil, the contactor being normally held open by a spring 59, or by its own weight.

40 In order to assure that the light beam from mirror 41 will not affect the photo-electric cell 45 when the mirror is in certain positions but will affect said cell when the mirror is in other positions, I provide the casing 40 with a front wall 40' and with a front opening 40'', as indicated in 45 Figs. 6, 7, and 8. When the mirror is in the position shown in Fig. 6, the light beams or rays from the mirror will be obstructed by the wall 40' so as not to affect the cell 45, and when the 50 mirror has moved a suitable distance, such as to the positions shown in Figs. 7 and 8, the light beam may be cast upon the cell 45 through the opening 40'' of the casing 40. In order to assure the concentration of the light beams or rays on 55 the photo-electric cell in all appropriate positions of mirror 41, I interpose lenses at 60 and 61 between the mirror and the cell to intercept the beam or light rays from the mirror and rectify them so that they will be directed upon the cell 60 in different positions of the mirror from the position of the latter shown in Fig. 6 to its positions shown in Figs. 7 and 8. The lenses are shown connected together by an interposed tube 62 through which the rays may pass from the mirror. 65 The tube 62 may be supported by casing 40 by means of a post 63, (Fig. 5). The lens 60 is shown having its convex surface opposing the mirror and the lens 61 has its convex surface opposing the photo-electric cell, whereby in different angular positions of the mirror, with respect to the lenses, the light beam or rays from the mirror will be caused to be directed against the cell, converging to a point at the cell window.

70 The operation may be described as follows: 75 Two pieces of strip metal of similar manufacture

to that of the strip A to be treated and bearing the structure desired to be obtained through the treatment of strip A may be placed in the passageways of the transformers 26 and 27. The primary coils of the transformers and the galvanometer field circuit are then closed at the switches *d* and 5 *e* to energize the circuits, and resistance *f* will be adjusted until the mirror 41 assumes a position to cast the beam upon the photo-electric cell, such as indicated in Fig. 7, for causing closing 10 of the respective circuits at the relays 54 and 48, whereby current will be caused to flow through the coil 5 of the furnace for heating the latter. The "standard" piece B is allowed to remain in the transformer 27, the other piece is removed 15 from the transformer 26 and the strip A to be treated extends from the furnace and is inserted in the transformer 26 and passed through the rolls 15 and 16 to the reel 14. Assuming that the standard piece B has been quenched from 1500° 20 F. and it is desired to have the strip A heated to 1500° F. as it travels, the motor 22 will be caused to operate to propel strip A when the temperature of the furnace has reached the desired degree, such as 1500° F. So long as the furnace temperature 25 remains constant and the strip A is heated and quenched as it travels to correspond in desired characteristics to those of the "standard" strip B, the circuit of the primary windings 28 and 29 and the bucked circuit of the secondaries 30 of the transformers will remain balanced and the galvanometer will cause the mirror to be in such a position as to cast the light beam through the lenses upon the photo-electric cell to maintain the relays closed at 54 and 48 to continue 35 the flow of current through the furnace coil 5. At such time, the quenched strip A passing through the secondary 28' and the "standard" piece B in secondary 29' correspond in the desired characteristics. Should the traveling strip 40 A, at some portion after quenching, as it passes through said secondary, vary from that of the standard piece, such as to require less heat, a differential will occur in the circuit of the secondaries 45 of the transformers, because of different characteristics between the "standard" piece and the said portion of the strip, thereby causing operation of the galvanometer to actuate the mirror and move the light beam from the photo-electric cell, as shown in Fig. 6. Thereupon the photo-electric cell circuit controlling the coil 55 will cease functioning and the spring 56 will cause the contactor 54 to break the circuit 57 whereupon the spring 59 will operate the contactor 48 to break the circuit of the line 11, 12 and the current will be broken from the furnace coil 5. The traveling strip A will continue to be heated by the remaining heat in the furnace to bring the strip substantially to the characteristics of the standard piece. When the net temperature of the 60 furnace drops, say 10° F., and the characteristics of the strip A correspond to the characteristics of the standard piece B, the circuit of the transformer secondaries will again be balanced and the galvanometer will operate the mirror 41 to 65 cause the light ray to fall on the photo-electric cell to cause closing of the contactor 54 at the circuit 57, whereupon the coil 58 will be energized and cause closing of the contactor 48 of the line circuit 11, 12 to restore the current to the 70 furnace coil 5 to continue heating of the latter. The operations described occur successively as variations in characteristics occur in the heated and quenched strip with respect to the characteristics of the standard piece B for required 75

treatment of the strip A as it travels. If the furnace temperature should rise above the proper degree and thereby change the characteristics of the heated and quenched strip A as compared to the standard piece B, the circuit of the secondaries 28' and 29' through the coil 33 of the galvanometer will be so changed as to cause operation of the mirror 41 to remove its light beam from the photo-electric cell, (Fig. 6), thereby de-  
 5 energizing coil 55 to cause break of circuit 57 to cause consequent breaking of circuit at switch 48 and shutting off of the current through coil 5 of the furnace until such time as the furnace sufficiently cools to cause the quenched strip A  
 10 to again correspond with the standard piece B, thereupon the circuit of the secondaries through coil 33 will be again balanced and cause the mirror to cast a light beam on cell 45 to cause closing of circuits at contactors 54 and 48 and to restore cur-  
 15 rent to coil 5. Should the furnace temperature remain absolutely constant, any structural differences inherent in the strip will become apparent and will be automatically compensated for to produce a uniform product. For example, if  
 20 portions of the hardened strip contain less carbide in solid solution, the hardening temperature applied to portions of strip A richer in dissolved carbide will yield a quenched product higher in permeability when applied to the portion leaner  
 25 in dissolved carbide, so that when such portion of the strip A (e. g. leaner in dissolved carbide in the pre-hardened state) passes through the trans-  
 30 former 26 after being quenched at the prevailing temperature, it will possess greater permeability  
 35 than the strip higher in dissolved carbides, and will cause the galvanometer light beam to be turned to fall on the photo-electric cell, as though the furnace temperature had fallen, or, in other words, as though the pre-hardened strip richer  
 40 in dissolved carbide had been quenched from a lower temperature. The action of the photo-  
 45 electric cell with the light beam upon it, will cause the operation of the contactors 54 and 48 to cause current to flow through the furnace coil 5 until that part of the strip A leaner in dissolved carbides passes through the furnace and upon arrival in the transformer 26 of the strip richer in dissolved carbides in the original state, the permeability of the quenched strip will be again de-  
 50 creased, and the galvanometer mirror will operate to cause the light beam to pass from the photo-  
 55 electric cell, thereby causing operation of the contactors 54 and 48 to break their circuits, to shut off the current flow to coil 5, to cause automatic cooling of the furnace, to compensate for the changed characteristics of the strip A being treated. The furnace temperature will be constantly altered to meet any changes in the continuity of the metallurgical characteristics within  
 60 the steel strip A as compared to the standard piece B. The resulting product will be substantially uniform since the hardening temperatures will have been controlled so as to produce a substantially uniform amount of carbide in solution in the steel strip A. The automatic temperature changes described may be secured quickly enough to maintain a high degree of uniformity within the strip A which constantly emerges from the hardening system, through use of a high-frequency induction furnace, which is unusually adaptable to rapid temperature alteration.

While I have described the construction and the operation as applied to hardening and chilling a strip A of steel, it will be understood that my invention may be utilized for tempering hardened

steel strips, as well as controlling annealing of ferrous metal strips, and quenching rates of hardened steel, and also for controlling the speed of travel of a strip through a machine of the character described. In the drawings, I have illus- 5 trated means for tempering the hardened and quenched strip as it travels from the furnace de-  
 10 scribed. The furnace 2' having a muffle 3' and conductor coil 5' connected with line conductors 8' and 9', similar in construction to that described with respect to the furnace 2, is shown mounted on frame 1, beyond the transformer 26, in alignment with said transformer, whereby the hardened and quenched strip A from furnace 2 will travel through the furnace 2' to be heated to the desired extent for tempering the hardened strip. At a suitable distance from the furnace 2' for cooling the strip A in its travel is a transformer 26' for passage of said strip, and at 27' is a trans-  
 15 former to receive a "standard" tempered piece B'. A galvanometer and mirror similar to those previously described is within a casing 40' and conductors 31' and 32' connect the movable coil of the galvanometer with the transformers 26' and 27' in manner previously described respecting cor- 20 responding parts. A photo-electric cell 45' is in position to receive a light beam from the mirror in casing 40'. An amplifier 47' and transformer 49', similar to the amplifier 47 and transformer 49, having the supply lines 53', and the conductors 46' and 51' of the photo-electric cell circuit, corresponding to the parts previously described, will control the circuit through the conductors 8' and 9' for the coil 5' in manner previously de- 25 scribed, and conductors at 38' supply the gal- 30 vanometer field. Switches and relays (such as d, 37, 48, and 54) for the corresponding circuits, as previously described, including means, such as solenoids like 58 and 55 to operate the associate contactors, together with other adjuncts previous- 35 ly set forth, will be supplied to complete the electric devices, whereby a normally balanced opposed circuit between the secondary windings of the 40 transformers 26' and 27' will be established.

A standard piece B', previously hardened and 45 tempered as desired, will be placed in the passageway of the transformer 27' to serve as a core therein, and the hardened and quenched strip will be passed through the muffle 3' and through the passageway of the transformer 26', as 50 illustrated in Fig. 1. Suitable high-frequency electric current will be supplied to the coil 5' to cause the muffle 3' to be heated by induction to the desired degree. The operation of the gal- 55 vanometer and its mirror in association with the photo-electric cell 45', will be similar to that previously described, in connection with the bucked circuit between the secondaries of the 60 transformers 26' and 27' for causing control of the flow of current through coil 5' for maintaining the required temperature of the muffle 3', in accordance with the characteristics of the tem- 65 pered strip A passing from the furnace 2' with respect to the characteristics of the standard piece B'. That is to say, so long as the charac- 70 teristics of the tempered portion of the strip A in the transformer 26' correspond to the characteristics of the standard piece B', the corresponding galvanometer mirror will be in position to maintain a beam on the photo-electric cell 45' to keep the muffle 3' at a desired temperature for standard operation. Should the temperature of the muffle 3' rise and change the then existing characteristics of the adjacent portion of the tem- 75 pered strip A, a differential will occur in the cir-

cuit of the secondaries of the transformers 26' and 27', causing the associate galvanometer to operate its mirror to remove the light beam from said cell, thereby causing the latter to cease functioning and the circuit to the coil 5' will be broken. The tempering of the strip will continue and when the temperature of the muffle 3' drops appropriately (and the characteristics of the tempered strip passing through the transformer 26' and the standard piece B' correspond) the galvanometer circuit will balance and the galvanometer will operate to cause the light beam to again fall on the cell 45' to cause flow of current through the coil 5', to restore heating to the latter. The operations described follow in succession as the tempered strip travels to maintain the tempering of the strip in substantial accord with the desired characteristics of the tempered standard piece B'.

In accordance with the arrangements set forth, a traveling steel strip may be hardened and quenched, and then tempered, successively in a continuous manner, and the finished tempered strip may be wound on the reel 14 in an expeditious and economical way, with the assurance that the hardening and the tempering of the strip will be throughout its length in accordance with the standards of hardness and tempering desired to have characteristics of hardness and temper substantially correspond to those of the standard pieces selected, such as B and B'.

While I have illustrated and described means for hardening and subsequently tempering a continuous strip of metal as it travels, it will be understood that a strip may be hardened without at the same time tempering it, or that a strip previously hardened elsewhere may be tempered by passing through a furnace 2'. An apparatus may be provided with a hardening furnace or heater and its adjuncts as described or with a tempering furnace or heater and its adjuncts described. It also will be understood that a strip may be passed through either of the furnaces or heaters described for annealing the strip in conjunction with a standard annealed piece in an appropriate transformer, whereby the circuit through the secondaries of two transformers, described will be controlled for controlling the temperature of the annealing furnace or heater in manner described with respect to hardening or tempering a metal strip. The invention also may be utilized to control quenching rates, or the speed of the metal strip in its travel through the heat-treating devices, or in any other way, which will constantly insure the continuous agreement of the strip being treated with the standard adopted. By the means described, the furnace may be quickly heated to the desired temperature and may be maintained approximately at such temperature because the supply current for the furnace may be turned on and off automatically in accordance with the correspondence of desired characteristics between the standard piece B or B' selected and the portion of the strip being treated, since the current flow will continue so long as the proper heat is applied to the strip in accordance with its electrical permeability or the characteristics utilized. When such permeability or characteristics vary from that of the standard piece in such a manner as to affect the desired treatment of the strip the current flow will be automatically turned off and on, as required, and the furnace control may thereby be secured automatically, and the temperature of the furnace may be quickly altered to meet any

changes in the continuity of metallurgical characteristics within the steel strip. It is distinguished from the previous practice of furnace control from an arbitrary, pre-determined temperature maintained by stationary thermo-couples within the furnace. The resulting product, according to my invention, is substantially uniform since the hardening or the tempering may be so controlled as to constantly produce a uniform amount of carbide in solution in a traveling steel strip, whereby to effect the desired results therein. This is effected because the automatic temperature changes described may be secured quickly enough to maintain a high degree of uniformity within the strip as it continues to emerge from the hardening and/or tempering system.

Having now described my invention, what I claim is:—

1. The method of heat-treating a ferrous metal strip consisting in continuously passing the strip successively through a heated zone and through a quenching zone, passing the heated and quenched portion of the strip through a balanced electrical field and varying the temperature of the heated zone to cause the required amount of heat to be applied to the strip as it travels through said zone by means of variations in the electrical permeability of said strip in said field.

2. The method of heat-treating a ferrous metal strip consisting in passing the strip through a heated zone to heat the strip, passing the strip through a quenching zone, passing the strip thereafter through electrically operative devices, and causing by means of a standard strip in said devices operation of the said devices to control the temperature of the heating zone.

3. The method of heating and quenching a ferrous metal strip consisting in passing the strip through a heating zone and through a quenching zone and varying the temperature of said heating zone in accordance with the variations in the electrical permeability of the quenched strip.

4. The method of hardening and tempering a ferrous metal strip consisting in passing the strip successively through a heating zone, a quenching zone and another heating zone, and varying the temperature of the first heating zone as the strip travels through said zone in accordance with the variations in the electrical permeability of said strip after being heated and quenched.

5. The method of hardening and tempering a ferrous metal strip consisting in passing the strip successively through a heating zone, a quenching zone, and another heating zone for tempering the strip, varying the temperature of the first named heating zone in accordance with the variations in the electrical permeability of the quenched strip, and varying the temperature of the second heating zone in accordance with the variations in the electrical permeability of the tempered strip.

6. The method of hardening and tempering a ferrous metal strip consisting in passing the strip successively through a heating zone, a quenching zone, and another heating zone for tempering the strip, varying the heat applied to the strip as it travels through the first named heating zone by means of variations in the electrical permeability of the strip after being heated and quenched, and varying the heat applied to the strip as it travels through the tempering zone by means of variations in the electrical permeability of the strip after tempering.

ALBERT R. STARGARDTER.